

No. 786,115.

PATENTED MAR. 28, 1905.

A. R. GROTH.

METHOD OF MAKING HANDLED GLASSWARE.

APPLICATION FILED NOV. 1, 1904.

*Fig. 1.*



*Fig. 2.*



*Fig. 3.*



WITNESSES

*L. R. Somers*  
*H. M. Corwin*

INVENTOR

*Albert R. Grotz*  
*by Becker & Beers*  
*his atty.*

## UNITED STATES PATENT OFFICE.

ALBERT R. GROTH, OF WELLSBURG, WEST VIRGINIA, ASSIGNOR OF ONE-HALF TO EAGLE GLASS AND MANUFACTURING COMPANY, OF WELLSBURG, WEST VIRGINIA, A CORPORATION OF WEST VIRGINIA.

## METHOD OF MAKING HANDLED GLASSWARE.

SPECIFICATION forming part of Letters Patent No. 786,115, dated March 28, 1905.

Application filed November 1, 1904. Serial No. 230,942.

To all whom it may concern:

Be it known that I, ALBERT R. GROTH, of Wellsburg, Brooke county, West Virginia, have invented a new and useful Method of Making Handled Glassware, of which the following is a full, clear, and exact description, reference being had to the accompanying drawings, forming part of this specification, in which—

10 Figure 1 is a vertical sectional view showing the pressing of the glass blank. Fig. 2 is a similar view showing the operation of chilling the blank in the blow-mold, and Fig. 3 is a similar view showing the blowing of the article in the blow-mold.

15 My invention relates to the manufacture of handled glassware, and is designed to overcome the difficulties heretofore experienced in making such articles.

20 If the handle is pressed with its lower end integral with the body of the blank, the glass will blow out very thin over this handle in the blow-mold and injure or destroy the article. If the handle is formed with its lower end totally disconnected with the blank-body, it will sag and become pinched between the parts of the blow-mold.

25 My invention overcomes these and other difficulties; and it consists, first, in pressing a handled blank with a greater thickness of wall at or adjacent to the lower end of the handle than in the other parts.

It further consists in pressing the handle with a small pin connection between it and the body, this pin being forced up into the handle during blowing.

30 It also consists in supporting the handle against sagging in inserting the blank in the blow-mold, in chilling the thicker portion of the glass blank when blowing, and, further, in the steps hereinafter described and claimed.

35 In carrying out my invention in connection with the apparatus of the drawings I first press a blank substantially as shown in the mold 2 of Fig. 1, this mold being cut away at the bottom of the handle portion, so as to

thicken the wall of the pressed blank 3, as shown at 4. The handle 5 does not extend at its lower end to the body of the blank; but a small connection or pin 6 is pressed which 50 connects these parts. The blank, which may otherwise be of any suitable shape, is then placed in the blow-mold 7, (shown in Fig. 2,) this blow-mold having a projecting pin 8 on one-half which acts to support the handle 55 against sagging during insertion and action in the mold. This projecting pin enters a corresponding recess in the other mold half when the parts are closed. After insertion and closing of the blow-mold the hand chilling and 60 pressing device 9 is inserted, this being in the form of an iron or steel plug having a suitable handle and preferably formed with an exit-channel 10 to allow the hot air to pass out from the blank. The operator inserts this 65 plug and then tilts it, as shown in Fig. 2, so as to chill the thicker portion of the glass below the handle to prevent its running down. This glass being thicker will retain its heat and be liable to droop or run down in the mold. 70 The presser may also act to partially force out this thicker wall toward the wall of the mold and partially shape the blank. After the chilling device is removed the blow-head 11 is applied to the mold and the article blown 75 out and expanded, as shown in Fig. 3 of the drawings.

The advantages of my invention result from the pressing of the blank with the thick wall below the handle to prevent excessive thinning of the wall at this point during expanding; also from the use of the small pin connection between the lower end of the handle and the body which holds the handle in position while the pin forces up into the handle 85 during expanding and prevents air entering which would make the handle hollow. The chilling of the thicker wall prevents drooping or running down, and the supporting of the handle avoids pinching it between the blow- 90 mold halves.

Many changes may be made in the form and

arrangement of the mold, shape of the article, the handle connections, &c., without departing from my invention.

I claim—

- 5 1. The method of forming handled glass-ware, consisting in pressing a hollow blank with a continuous wall having a thickened portion under the lower end of the handle, and then expanding the lower part of the hol-  
10 low blank to final form; substantially as de-scribed.
2. The method of making handled glass-ware, consisting in pressing a blank with a small pin connection between the lower end  
15 of the handle and the blank, and then expand-ing the blank to final form; substantially as de-scribed.
3. The method of forming handled glass-ware, consisting in pressing a blank with a  
20 thick wall on one or more sides and a small pin connection between said walls, and the lower end of the handle, then expanding the blank, and forcing the pin upwardly into the lower end of the handle; substantially as de-  
25 scribed.
4. The method of forming handled glass-ware, consisting in pressing a blank with a

thicker wall beneath the handle, chilling this thicker portion, and then expanding the blank; substantially as described.

30

5. The method of forming handled glass-ware, consisting in pressing a blank with a thicker wall beneath the handle, chilling and partially expanding this thicker portion, and then expanding the blank; substantially as de-  
35 scribed.

6. The method of forming handled glass-ware, consisting in pressing a hollow blank with an integral handle, inserting the blank in a blow-mold, and supporting the handle  
40 against sagging, and then blowing the blank to final form; substantially as described.

7. The method of forming handled glass-ware, consisting in pressing a blank with a bridge connection between the lower end of  
45 the handle and the blank-body, and then ex-panding the body in a blow-mold; substan-tially as described.

In testimony whereof I have hereunto set my hand.

ALBERT R. GROTH.

Witnesses:

JAMES PAINE,  
MINNIE E. LINTON.